# EUROPEAN PATENT SPECIFICATION

(11) **EP 0 710 730 B1**
(45) Date of publication and mention of the grant of the patent: **02.10.2002**
(21) Application number: 95117263.4
(22) Date of filing: 02.11.1995
(51) Int. Cl.: C22C 21/00, B22F 9/06, C23C 26/00

(54) **High strength and high rigidity aluminium based alloy and production method therefor**
Hochfeste und hochsteife Aluminiumbasislegierung und deren Herstellungsverfahren
Alliage à base d'aluminium à haute résistance mécanique et à haute rigidité et sa méthode de fabrication

(30) Priority: 02.11.1994 JP 27006294
(43) Date of publication of application: 08.05.1996
(73) Proprietor: Masumoto, Tsuyoshi, Sendai-shi, Miyagi-ken (JP); Inoue, Akihisa, Sendai-shi, Miyagi-ken (JP); YAMAHA CORPORATION, Hamamatsu-shi, Shizuoka-ken 430 (JP)
(72) Inventor: Inoue, Akihisa, Sendai-shi, Miyagi-ken (JP); Kimura, Hisamichi, Watari-gun, Miyagi-ken (JP); Horio, Yuma, c/o Yamaha Corp., Hamamatsu-shi, Shizuoka-ken (JP)
(74) Representative: Geyer, Ulrich F., Dr. Dipl.-Phys.

(56) References cited:
- EP-A- 0 584 596
- EP-A- 0 587 186
- SIXTH INTERNATIONAL CONFERENCE ON RAPIDLY QUENCHED METALS, MONTREAL, QUE., CANADA, 3-7 AUG. 1987, vol. 99, ISSN 0025-5416, MATERIAL SCIENCE AND ENGINEERING, MARCH 1988, SWITZERLAND, pages 407-411, XP000600857 SKINNER D J ET AL: "Stability of quasicrystalline phases in Al-Fe-V"
- EIGHTH INTERNATIONAL CONFERENCE ON RAPIDLY QUENCHED AND METASTABLE MATERIALS, SENDAI, JAPAN, 22-27 AUG. 1993, vol. A179-A180, ISSN 0921-5093, MATERIALS SCIENCE & ENGINEERING A (STRUCTURAL MATERIALS: PROPERTIES, MICROSTRUCTURE AND PROCESSING), 1 MAY 1994, SWITZERLAND, pages 665-668, XP000600949 ANDERSEN S J ET AL: "Microstructure of rapidly solidified Al-7.5Cu-2.5Fe"
- Inspec abstracts AN=3224108 and AN=4146829
- DATABASE INSPEC, , INSPEC no. 3224108, DUNLAP R. A. ET AL.: "Physical properties of a rapidly quenched Al-Fe alloys",
- DATABASE INSPEC, , INSPEC no. 4146829, KIM D. H. ET AL.: "A study on the microstructural characteristics of rapidly solidified Al-Fe alloys. II. quasicrystalline and related crystalline phase",

## Description

### BACKGROUND OF THE INVENTION

### Field of the Invention

The present invention relates to an aluminum-based alloy for use in a wide range of applications such as in a structural material for aircraft, vehicles, and ships, and for engine parts. In addition, the present invention may be employed in sashes, roofing materials, and exterior materials for use in construction, or as material for use in marine equipment, nuclear reactors, and the like.

### Description of Related Art

As prior art aluminum-based alloys, alloys incorporating various components such as Al-Cu, Al-Si, Al-Mg, Al-Cu-Si, Al-Cu-Mg, and Al-Zn-Mg are known. In all of the aforementioned, superior anti-corrosive properties are obtained at a light weight, and thus the aforementioned alloys are being widely used as structural material for machines in vehicles, ships, and aircraft, in addition to being employed in sashes, roofing materials, exterior materials for use in construction, structural material for use in LNG tanks, and the like.

However, the prior art aluminum-based alloys generally exhibit disadvantages such as a low hardness and poor heat resistance when compared to material incorporating Fe. In addition, although some materials have incorporated elements such as Cu, Mg, and Zn for increased hardness, disadvantages remain such as low anti-corrosive properties.

On the other hand, recently, experiments have been conducted in which a fine metallographic structure of aluminum-based alloys is obtained by means of performing quick-quench solidification from a liquid-melt state, resulting in the production of superior mechanical strength and anti-corrosive properties.

In Japanese Patent Application, First Publication No. 1-275732, an aluminum-based alloy comprising a composition AlM₁X with a special composition ratio (wherein M₁ represents an element such as V, Cr, Mn, Fe, Co, Ni, Cu, Zr and the like, and X represents a rare earth element such as La, Ce, Sm, and Nd, or an element such as Y, Nb, Ta, Mm (misch metal) and the like), and having an amorphous or a combined amorphous/fine crystalline structure, is disclosed.

This aluminum-based alloy can be utilized as material with a high hardness, high strength, high electrical resistance, anti-abrasion properties, or as soldering material. In addition, the disclosed aluminum-based alloy has a superior heat resistance, and may undergo extruding or press processing by utilizing the superplastic phenomenon observed near crystallization temperatures.

However, the aforementioned aluminum-based alloy is disadvantageous in that high costs result from the incorporation of large amounts of expensive rare earth elements and/or metal elements with a high activity such as Y. Namely, in addition to the aforementioned use of expensive raw materials, problems also arise such as increased consumption and labor costs due to the large scale of the manufacturing facilities required to treat materials with high activities. Furthermore, this aluminum-based alloy having the aforementioned composition tends to display insufficient resistance to oxidation and corrosion.

EP-A-584 596 relates to a high strength aluminum-based alloy essentially consisting of an amorphous structure or a multiphase amorphous/fine crystalline structure.

Further, Skinner et al. in "Stability of Quasicrystalline Phases in Al-Fe-V Alloys," Mat. Sci. and Eng., 99, 1988, pp. 407-411, disclose Al-V-Fe quasi-crystalline alloys produced by melt spinning techniques, and thermal stability and microstructures thereof.

Dunlap et al. in "Physical properties of a rapidly quenched Al-Fe alloys", J. Phys. F, Met. Phys., July 1988, UK, pp. 1329-1341, and Kim et al. in "Microstructural characteristics of rapidly solidified Al-Fe alloys. II. Quaiscrystalline and related crystalline phase," J. Korean Inst. Met. (South Korea), Sept. 1991, South Korea, pp. 976-982, disclose binary Al-Fe quasi-crystalline alloys.

### SUMMARY OF THE INVENTION

It is an object of the present invention to provide an aluminum-based alloy, possessing superior strength, rigidity, and anti-corrosive properties, which comprises a composition in which rare earth elements or high activity elements such as Y are not incorporated, thereby effectively reducing the cost, as well as, the activity described in the aforementioned.

In order to solve the aforementioned problems, the present invention provides a high strength and high rigidity aluminum-based alloy according the features of claim 1.

According to the present invention, by adding a predetermined amount of V, Mo, Fe, W, Nb, and/or Pd to Al, the ability of the alloy to form a quasi-crystalline phase is improved, and the strength, hardness, and toughness of the alloy is also improved. Moreover, by adding a predetermined amount of Mn, Fe, Co, Ni, and/or Cu, the effects of quick-quenching are enhanced, the thermal stability of the overall metallographic structure is improved, and the strength and hardness of the resulting alloy are also increased.

The aluminum-based alloy according to the present invention is useful as materials with a high hardness, strength, and rigidity. Furthermore, this alloy also stands up well to bending, and thus possesses superior properties such as the ability to be mechanically processed.

Accordingly, the aluminum-based alloys according to the present invention can be used in a wide range of applications such as in the structural material for aircraft, vehicles, and ships, as well as for engine parts. In addition, the aluminum-based alloys of the present invention may be employed in sashes, roofing materials, and exterior materials for use in construction, or as materials for use in marine equipment, nuclear reactors, and the like.

### BRIEF DESCRIPTION OF THE DRAWINGS

Fig. 1 shows a construction of an example of a single roll apparatus used at the time of manufacturing a tape of an alloy of the present invention following quick-quench solidification.

Fig. 2 shows the analysis result of the x-ray diffraction of an alloy having the composition of Al₉₄V₄Fe₂.

Fig. 3 shows the analysis result of the X-ray diffraction of an alloy having the composition of Al₉₅Mo₃Ni₂.

Fig. 4 shows the analysis result of the X-ray diffraction of an alloy having the composition of Al₉₁Nb₆Co₃.

Fig. 5 shows the thermal properties of an alloy having the composition of Al₉₄V₄Ni₂.

### DETAILED DESCRIPTION OF THE PREFERRED EMBODIMENTS

The first preferred embodiment of the present invention provides a high strength and high rigidity aluminum-based alloy consisting essentially of a composition represented by the general formula Al_{100-(a+b)}QₐM_{b} (wherein Q is at least one metal element selected from the group consisting of V, Mo, Fe, W, Nb, and Pd; M is at least one metal element selected from the group consisting of Mn, Fe, Co, Ni, and Cu; and a and b, which represent a composition ratio in atomic percentages, satisfy the relationships 1 ≤ a ≤ 10, 0 < b < 5, and 3 ≤ a+b ≤ 12), comprising a quasi-crystalline phase in the alloy.

In the following, the reasons for limiting the composition ratio of each component in the alloy according to the present invention are explained.

The atomic percentage of Al (aluminum) is in the range of 88 ≤ Al ≤ 97, preferably in the range of 92 ≤ Al ≤ 97, and more preferably in the range of 94 ≤ Al ≤ 97. An atomic percentage for Al of less than 88% results in embrittlement of the alloy. On the other hand, an atomic percentage for Al exceeding 97% results in reduction of the strength and hardness of the alloy.

The amount of at least one metal element selected from the group consisting of V (vanadium), Mo (molybdenum), Fe (iron), W (tungsten), Nb (niobium), and Pd (palladium) in atomic percentage is at least 1% and does not exceed 10%; preferably, the amount is at least 2% and does not exceed 8%; more prefarably, the amount is at least 2% and does not exceed 6%. If the amount is less than 1%, a quasi-crystalline phase cannot be obtained, and the strength is markedly reduced. On the other hand, if the amount exceeds 10%, coarsening (the diameter of particles is 500 nm or more) of a quasi-crystalline phase occurs, and this results in remarkable embrittlement of the alloy and reduction of (rupture) strength of the alloy.

The amount of at least one metal element selected from the group consisting of Mn (manganese), Fe (iron), Co (cobalt), Ni (nickel), and Cu (copper) in atomic percentage is less than 5%; preferably, the amount is at least 1% and does not exceed 3%; more preferably, the amount is at least 1% and does not exceed 2%. If the amount is 5% or more, forming and coarsening (the diameter of particles is 500 nm or more) of intermetallic compounds occur, and these result in remarkable embrittlement and reduction of toughness of the alloy.

Furthermore, the total amount of unavoidable impurities, such as Fe (if not a selected metal element), Si, Cu (if not a selected metal element), Zn, Ti, O, C, or N, does not exceed 0.3% by weight; preferably, the amount does not exceed 0.15% by weight; and more preferably, the amount does not exceed 0.10% by weight. If the amount exceeds 0.3% by weight, the effects of quick-quenching is lowered, and this results in reduction of the formability of a quasi-crystalline phase. Among the unavoidable impurities, particularly, it is preferable that the amount of O does not exceed 0.1% by weight and that the amount of C or N does not exceed 0.03% by weight.

The aforementioned aluminum-based alloys can be manufactured by quick-quench solidification of the alloy liquid-melts having the aforementioned compositions using a liquid quick-quenching method. This liquid quick-quenching method essentially entails rapid cooling of the melted alloy. For example, single roll, double roll, and submerged rotational spin methods have proved to be particularly effective. In these aforementioned methods, a cooling rate of 10⁴ to 10⁶ K/sec is easily obtainable.

In order to manufacture a thin tape using the aforementioned single or double roll methods, the liquid-melt is first poured into a storage vessel such as a silica tube, and is then discharged, via a nozzle aperture at the tip of the silica tube, towards a copper or copper alloy roll of diameter 30 to 300 mm, which is rotating at a fixed velocity in the range of 300 to 1000 rpm. In this manner, various types of thin tapes of thickness 5 - 500 µm and width 1 - 300 mm can be easily obtained.

On the other hand, fine wire-thin material can be easily obtained through the submerged rotational spin method by discharging the liquid-melt via the nozzle aperture, into a refrigerant solution layer of depth 1 to 10 cm, maintained by means of centrifugal force inside an air drum rotating at 50 to 500 rpm, under argon gas back pressure. In this case, the angle between the liquid-melt discharged from the nozzle, and the refrigerant surface is preferably 60 to 90 degrees, and the relative velocity ratio of the liquid-melt and the refrigerant surface is preferably 0.7 to 0.9.

In addition, thin layers of aluminum-based alloy of the aforementioned compositions can also be obtained without using the above methods, by employing layer formation processes such as the sputtering method. In addition, aluminum alloy powder of the aforementioned compositions can be obtained by quick-quenching the liquid-melt using various atomizer and spray methods such as a high pressure gas spray method.

In the following, examples of metallographic-structural states of the aluminum-based alloy obtained using the aforementioned methods are listed:
(1) Multiphase structure incorporating a quasi-crystalline phase and an aluminum phase;
(2) Multiphase structure incorporating a quasi-crystalline phase and a metal solid solution having an aluminum matrix;
(3) Multiphase structure incorporating a quasi-crystalline phase and a stable or metastable intermetallic compound phase; and
(4) Multiphase structure incorporating a quasi-crystalline phase, an amorphous phase, and a metal solid solution having an aluminum matrix.

A widely-recognized definition of "quasi-crystalline" is given for a structure satisfying the following three conditions with respect to the reciprocal lattice or diffraction pattern:
(A) the diffraction pattern consists of a set of δ-functions (or points);
(B) the number of fundamental unit vectors describing the distribution of the reciprocal lattice points (diffraction particles) must be greater than the number of dimensions (i.e., equal to or greater than four for an actual quasi-crystal); and
(C) the structure has a rotation symmetry which is not permitted for a crystal. (It should be noted that a crystal has only one-, two-, three-, four-, or six-folded rotation symmetry.)

Condition (A) may be satisfied by a crystal.

In the case of a crystal, when three short, independent diffraction vectors *a*, b**, and *c** are chosen as the fundamental vectors as in Condition (B), all diffraction points can be formulated as a linear combination of the three vectors, namely, the formula *la**+*mb**+*nc**. However, since more than three fundamental unit vectors are necessary for an incommensurate crystal, a material cannot be identified as a quasi-crystal by merely satisfying Conditions (A) and (B). Thus, a quasi-crystal must meet also Condition (C).

(When a lattice is modulated by a period *a'* which differs from the natural period *a*, if the value *a*'/*a* is an irrational number, such a crystal is called an "incommensurate crystal". Such a modulation occurs when re-distribution of electrons, such as charge density wave, affects the lattice.)

The above definition of quasi-crystal relates to reciprocal lattices. Therefore, examination of diffraction patterns in detail allows experimental judgement as to whether or not a material is a quasi-crystal.

Specifically, quasi-crystals having a five-fold rotation symmetry are known. As quasi-crystalline phases defined in the above, regular icosahedral phase, regular decagonal phase, regular dodecagonal phase, and regular octagonal phase have been found.

A quasi-crystal was first discovered by Shechtmann, et al., of Israel in 1984. This quasi-crystal was of the regular icosahedral phase (D. Shechtmann, I. A. Blech, D. Gratias, and J. W. Cahn; Phys. Rev. Lett., **53** (1984), 1951).

The fine crystalline phase of the present invention represents a crystalline phase in which the crystal particles have an average maximum diameter of 1 µm.

By regulating the cooling rate of the alloy liquid-melt, any of the metallographic-structural states described in (1) to (4) above can be obtained.

The properties of the alloys possessing the aforementioned metallographic-structural states are described in the following.

An alloy of the multiphase structural state described in (1) and (2) above has a high strength and an excellent bending ductility.

An alloy of the multiphase structural state described in (3) above has a higher strength and lower ductility than the alloys of the multiphase structural state described in (1) and (2). However, the lower ductility does not hinder its high strength.

An alloy of the multiphase structural state described in (4) has a high strength, high toughness and a high ductility.

Each of the aforementioned metallographic-structural states can be easily determined by a normal X-ray diffraction method or by observation using a transmission electron microscope. In the case when a quasi-crystal exists, a dull peak, which is characteristic of a quasi-crystalline phase, is exhibited.

By regulating the cooling rate of the alloy liquid-melt, any of the multiphase structural states described in (1) to (3) above can be obtained.

By quick-quenching the alloy liquid-melt of the Alrich composition (e.g., composition with Al ≥ 92 atomic %), any of the metallographic-structural states described in (4) can be obtained.

The aluminum-based alloy of the present invention displays superplasticity at temperatures near the crystallization temperature (crystallization temperature ±50°C), as well as, at the high temperatures within the fine crystalline stable temperature range, and thus processes such as extruding, pressing, and hot forging can easily be performed. Consequently, aluminum-based alloys of the above-mentioned compositions obtained in the aforementioned thin tape, wire, plate, and/or powder states can be easily formed into bulk materials by means of extruding, pressing and hot forging processes at the aforementioned temperatures. Furthermore, the aluminum-based alloys of the aforementioned compositions possess a high ductility, thus bending of 180° is also possible.

Additionally, the aforementioned aluminum-based alloys having multiphase structure composed of a pure-aluminum phase, a quasi-crystalline phase, a metal solid solution, and/or an amorphous phase, and the like, do not display structural or chemical non-uniformity of crystal grain boundary, segregation and the like, as seen in crystalline alloys. These alloys cause passivation due to formation of an aluminum oxide layer, and thus display a high resistance to corrosion. Furthermore, disadvantages exist when incorporating rare earth elements: due to the activity of these rare earth elements, non-uniformity occurs easily in the passive layer on the alloy surface resulting in the progress of corrosion from this portion towards the interior. However, since the alloys of the aforementioned compositions do not incorporate rare earth elements, these aforementioned problems are effectively circumvented.

In regards to the aluminum-based alloy of the aforementioned compositions, the manufacturing of bulk-shaped (mass) material will now be explained.

When heating the aluminum-based alloy according to the present invention, precipitation and crystallization of the fine crystalline phase is accompanied by precipitation of the aluminum matrix (α-phase), and when further heating beyond this temperature, the intermetallic compound also precipitates. Utilizing this property, bulk material possessing a high strength and ductility can be obtained.

Concretely, the tape alloy manufactured by means of the aforementioned quick-quenching process is pulverized in a ball mill, and then powder pressed in a vacuum hot press under vacuum (e.g. 10⁻³ Torr) at a temperature slightly below the crystallization temperature (e.g. approximately 470K), thereby forming a billet for use in extruding with a diameter and length of several centimeters. This billet is set inside a container of an extruder, and is maintained at a temperature slightly greater than the crystallization temperature for several tens of minutes. Extruded materials can then be obtained in desired shapes such as round bars, etc., by extruding.

### Examples

A molten alloy having a predetermined composition was manufactured using a high frequency melting furnace. Then, as shown in Fig. 1, this melt was poured into a silica tube 1 with a small aperture 5 (aperture diameter: 0.2 to 0.5 mm) at the tip, and then heated to melt, after which the aforementioned silica tube 1 was positioned directly above copper roll 2. This roll 2 was then rotated at a high speed of 4000 rpm, and argon gas pressure (0.7 kg/cm³) was applied to silica tube 1. Quick-quench solidification was subsequently performed by quick-quenching the liquid-melt by means of discharging the liquid-melt from small aperture 5 of silica tube 1 onto the surface of roll 2 and quick-quenching to yield an alloy tape 4.

Under these manufacturing conditions, the numerous alloy tape samples (width: 1 mm, thickness: 20 µm) of the compositions (atomic percentages) shown in Tables 1 and 2 were formed. The hardness (Hv) and tensile rupture strength (σ_{f}: MPa) of each alloy tape sample were measured. These results are also shown in Tables 1 and 2. The hardness is expressed in the value measured according to the minute Vickers hardness scale (DPN: Diamond Pyramid Number).

Additionally, a 180° contact bending test was conducted by bending each sample 180° and contacting the ends thereby forming a U-shape. The results of these tests are also shown in Tables 1 and 2: those samples which displayed ductility and did not rupture are designated Duc (ductile), while those which ruptured are designated Bri (brittle).

**Table 1**

| Sample No. | Alloy composition (at%) | σf (MPa) | Hv (DPN) | Bending test | |
|---|---|---|---|---|---|
| 1 | Al₉₅V₃Ni₂ | 880 | 320 | Duc | Example |
| 2 | Al₉₄V₄Ni₂ | 1230 | 365 | Duc | Example |
| 3 | Al₉₃V₅Ni₂ | 1060 | 325 | Duc | Example |
| 4 | Al₉₅V₃Fe₂ | 630 | 300 | Duc | Example |
| 5 | Al₉₄V₄Fe₂ | 1350 | 370 | Duc | Example |
| 6 | Al₉₃V₅Fe₂ | 790 | 305 | Duc | Example |
| 7 | Al₉₅V₃Co₂ | 840 | 310 | Duc | Example |
| 8 | Al₉₄V₄Co₂ | 1230 | 355 | Duc | Example |
| 9 | Al₉₃V₅Co₂ | 1090 | 350 | Duc | Example |
| 10 | Al₉₄V₄Mn₂ | 1210 | 355 | Duc | Example |
| 11 | Al₉₁V₈Mn₂ | 1010 | 345 | Duc | Example |
| 12 | Al₉₃V₄Mn₃ | 800 | 310 | Duc | Example |
| 13 | Al₉₄V₄Cu₂ | 1010 | 310 | Duc | Example |
| 14 | Al₈₈V₁₀Cu₂ | 810 | 305 | Duc | Example |
| 15 | Al₈₈V₈Cu₄ | 650 | 295 | Duc | Example |
| 16 | Al₈₉V₁₀Ni₁ | 840 | 310 | Duc | Example |
| 17 | Al₉₂V₅Ni₃ | 1110 | 330 | Duc | Example |
| 18 | Al₉₃V₄Fe₃ | 1200 | 340 | Duc | Example |
| 19 | Al₉₃V₆Fe₁ | 1210 | 345 | Duc | Example |
| 20 | Al₉₂V₇Co₁ | 1010 | 310 | Duc | Example |
| 21 | Al₉₃V₄Co₃ | 1110 | 310 | Duc | Example |
| 22 | Al₉₄Mo₄Ni₂ | 1200 | 300 | Duc | Example |
| 23 | Al₉₅Mo₃Ni₂ | 1250 | 305 | Duc | Example |
| 24 | Al₉₃Mo₅Ni₂ | 1300 | 320 | Duc | Example |
| 25 | Al₉₄Mo₄Co₂ | 1010 | 300 | Duc | Example |
| 26 | Al₈₉Mo₈Co₃ | 1010 | 305 | Duc | Example |
| 27 | Al₉₅Mo₃Co₂ | 1210 | 330 | Duc | Example |
| 28 | Al₉₃Mo₅Fe₂ | 990 | 310 | Duc | Example |
| 29 | Al₉₀Mo₇Fe₃ | 1110 | 320 | Duc | Example |
| 30 | Al₉₄Mo₄Fe₂ | 1320 | 375 | Duc | Example |
| 31 | Al₉₄Mo₄Mn₂ | 1220 | 360 | Duc | Example |
| 32 | Al₉₂Mo₅Mn₃ | 1100 | 345 | Duc | Example |
| 33 | Al₉₅Mo₃Mn₂ | 1020 | 330 | Duc | Example |
| 34 | Al₉₇Mo₁Cu₂ | 880 | 305 | Duc | Example |
| 35 | Al₈₉Mo₁₀Cu₁ | 890 | 300 | Duc | Example |
| 36 | Al₉₀Mo₇Cu₃ | 880 | 300 | Duc | Example |
| 37 | Al₉₄Fe₄Mn₂ | 1320 | 370 | Duc | Example |
| 38 | Al₉₄Fe₃Mn₃ | 1100 | 345 | Duc | Example |
| 39 | Al₉₁Fe₈Mn₁ | 1210 | 365 | Duc | Example |
| 40 | Al₉₄Fe₄Co₂ | 1310 | 370 | Duc | Example |
| 41 | Al₉₄Fe₅Co₁ | 1110 | 335 | Duc | Example |
| 42 | Al₉₆Fe₃Co₁ | 1010 | 320 | Duc | Example |
| 43 | Al₉₀Fe₈Ni₂ | 1100 | 340 | Duc | Example |
| 44 | Al₈₈Fe₁₀Ni₂ | 1300 | 375 | Duc | Example |
| 45 | Al₈₈Fe₉Ni₃ | 1280 | 360 | Duc | Example |
| 46 | Al₉₄Fe₄Cu₂ | 890 | 285 | Duc | Example |
| 47 | Al₉₅Fe₄Cu₁ | 880 | 300 | Duc | Example |
| 48 | Al₈₈Fe₈Cu₃ | 930 | 295 | Duc | Example |
| 49 | Al₉₄W₄Ni₂ | 1010 | 340 | Duc | Example |
| 50 | Al₈₉W₈Ni₃ | 990 | 310 | Duc | Example |
| 51 | Al₉₄W₃Ni₃ | 1000 | 300 | Duc | Example |
| 52 | Al₉₃W₅Co₂ | 1110 | 315 | Duc | Example |
| 53 | Al₉₅W₂Co₃ | 1210 | 365 | Duc | Example |
| 54 | Al₉₄W₄Fe₂ | 1090 | 305 | Duc | Example |
| 55 | Al₉₃W₆Fe₁ | 1100 | 360 | Duc | Example |
| 56 | Al₉₀W₈Fe₂ | 1060 | 340 | Duc | Example |
| 57 | Al₉₁W₅Mn₄ | 1130 | 345 | Duc | Example |
| 58 | Al₉₄W₂Mn₄ | 1210 | 350 | Duc | Example |
| 59 | Al₉₀W₈Cu₂ | 910 | 310 | Duc | Example |
| 60 | Al₉₀W₇Cu₃ | 890 | 305 | Duc | Example |
| 61 | Al₉₀Nb₆Mn₄ | 1160 | 335 | Duc | Example |
| 62 | Al₉₀Nb₇Mn₃ | 1070 | 320 | Duc | Example |
| 63 | Al₉₂Nb₆Mn₂ | 1230 | 330 | Duc | Example |
| 64 | Al₉₄Nb₄Fe₂ | 1040 | 320 | Duc | Example |
| 65 | Al₉₁Nb₈Fe₁ | 1110 | 340 | Duc | Example |
| 66 | Al₉₀Nb₇Fe₃ | 890 | 305 | Duc | Example |
| 67 | Al₉₄Nb₄Ni₂ | 1300 | 370 | Duc | Example |
| 68 | Al₉₃Nb₃Ni₄ | 1210 | 360 | Duc | Example |
| 69 | Al₉₅Nb₃Ni₂ | 1100 | 360 | Duc | Example |
| 70 | Al₉₄Nb₄Co₂ | 1150 | 365 | Duc | Example |
| 71 | Al₉₀Nb₇Co₃ | 1160 | 345 | Duc | Example |
| 72 | Al₉₁Nb₆Co₃ | 1020 | 335 | Duc | Example |
| 73 | Al₉₀Nb₈Cu₂ | 990 | 320 | Duc | Example |
| 74 | Al₂₀Nb₆Cu₄ | 900 | 300 | Duc | Example |
| 75 | Al₉₀Nb₈Cu₂ | 930 | 305 | Duc | Example |
| 76 | Al₉₁Pd₆Mn₃ | 1020 | 320 | Duc | Example |
| 77 | Al₉₁Pd₇Mn₂ | 1270 | 345 | Duc | Example |
| 78 | Al₉₀Pd₈Mn₂ | 1190 | 320 | Duc | Example |
| 79 | Al₉₄Pd₄Fe₂ | 1010 | 315 | Duc | Example |
| 80 | Al₆Pd₃Fe₁ | 990 | 310 | Duc | Example |
| 81 | Al₉₀Pd₆Fe₄ | 1010 | 325 | Duc | Example |
| 82 | Al₉₀Pd₈Ni₂ | 1100 | 340 | Duc | Example |
| 83 | Al₉₄Pd₄Ni₂ | 1210 | 365 | Duc | Example |
| 84 | Al₉₂Pd₅Ni₃ | 1230 | 365 | Duc | Example |
| 85 | Al₉₄Pd₃Co₃ | 1100 | 335 | Duc | Example |
| 86 | Al₉₁Pd₆Co₃ | 1260 | 360 | Duc | Example |
| 87 | Al₈₉Pd₈Co₃ | 1000 | 340 | Duc | Example |
| 88 | Al₉₁Pd₇Cu₁ | 980 | 300 | Duc | Example |
| 89 | Al₈₈Pd₉Cu₃ | 970 | 295 | Duc | Example |
| 90 | Al₉₀Pd₈Cu₂ | 990 | 300 | Duc | Example |

**Table 2**

| Sample No. | Alloy composition (at%) | σf (MPa) | Hv (DPN) | Bending test | |
|---|---|---|---|---|---|
| 91 | Al_{96.5}V_{0.5}Mn₃ | 460 | 95 | Duc | Comparative Example |
| 92 | Al₈₆V₁₂Mn₂ | 600 | 450 | Bri | Comparative Example |
| 93 | Al₉₇V₃ | 400 | 120 | Duc | Comparative Example |
| 94 | Al₉₀V₄Mn₆ | 550 | 410 | Bri | Comparative Example |
| 95 | Al₉₈V₁Mn₁ | 430 | 95 | Duc | Comparative Example |
| 96 | Al₈₇V₁₀Mn₃ | 510 | 410 | Bri | Comparative Example |
| 97 | Al_{96.5}V_{0.5}Fe₃ | 410 | 120 | Duc | Comparative Example |
| 98 | Al₈₅V₁₃Fe₂ | 505 | 405 | Bri | Comparative Example |
| 99 | Al₉₈V₁Fe₁ | 400 | 110 | Duc | Comparative Example |
| 100 | Al₈₇V₁₀Fe₃ | 490 | 410 | Bri | Comparative Example |
| 101 | Al₉₀V₄Fe₆ | 450 | 430 | Bri | Comparative Example |
| 102 | Al_{95.5}V_{0.5}Ni₄ | 390 | 95 | Duc | Comparative Example |
| 103 | Al₈₆V₁₁Ni₃ | 410 | 430 | Bri | Comparative Example |
| 104 | Al₈₉V₄Ni₇ | 405 | 425 | Bri | Comparative Example |
| 105 | Al₉₈V₁Ni₁ | 290 | 80 | Duc | Comparative Example |
| 106 | Al₈₅V₁₁Ni₄ | 500 | 420 | Bri | Comparative Example |
| 107 | Al_{94.5}V_{0.5}Co₅ | 410 | 125 | Duc | Comparative Example |
| 108 | Al₈₃V₁₅Co₂ | 490 | 480 | Bri | Comparative Example |
| 109 | Al₉₀V₂Co₆ | 480 | 410 | Bri | Comparative Example |
| 110 | Al_{98.5}V_{0.5}Co₁ | 210 | 90 | Duc | Comparative Example |
| 111 | Al₈₅V₁₁Co₄ | 410 | 430 | Bri | Comparative Example |
| 112 | Al_{94.5}V_{0.5}Cu₅ | 340 | 105 | Duc | Comparative Example |
| 113 | Al₈₈V₁₁Cu₁ | 490 | 420 | Bri | Comparative Example |
| 114 | Al₈₉V₃Cu₈ | 480 | 410 | Bri | Comparative Example |
| 115 | Al₉₈V₁Cu₁ | 410 | 95 | Duc | Comparative Example |
| 116 | Al₈₅V₁₂Cu₃ | 550 | 420 | Bri | Comparative Example |
| 117 | Al_{96.5}Mo_{0.5}Mn₃ | 430 | 125 | Duc | Comparative Example |
| 118 | Al₈₆Mo₁₂Mn₂ | 510 | 430 | Bri | Comparative Example |
| 119 | Al₉₇Mo₃ | 370 | 130 | Duc | Comparative Example |
| 120 | Al₉₀Mo₄Mn₆ | 480 | 410 | Bri | Comparative Example |
| 121 | Al₉₈Mo₁Mn₁ | 380 | 100 | Duc | Comparative Example |
| 122 | Al₈₇Mo₁₀Mn₃ | 490 | 420 | Bri | Comparative Example |
| 123 | Al_{96.5}Mo_{0.5}Fe₃ | 360 | 125 | Duc | Comparative Example |
| 124 | Al₈₅Mo₁₃Fe₂ | 500 | 460 | Bri | Comparative Example |
| 125 | Al₄₈Mo₁Fe₁ | 210 | 80 | Duc | Comparative Example |
| 126 | Al₈₇Mo₁₀Fe₃ | 510 | 450 | Bri | Comparative Example |
| 127 | Al₉₀Mo₄Fe₆ | 490 | 435 | Bri | Comparative Example |
| 128 | Al_{95.5}Mo_{0.5}Ni₄ | 310 | 95 | Duc | Comparative Example |
| 129 | Al₈₆Mo₁₁Ni₃ | 500 | 430 | Bri | Comparative Example |
| 130 | Al₈₉Mo₄Ni₇ | 465 | 410 | Bri | Comparative Example |
| 131 | Al₉₈Mo₁Ni₁ | 200 | 95 | Duc | Comparative Example |
| 132 | Al₈₅Mo₁₁Ni₄ | 460 | 450 | Bri | Comparative Example |
| 133 | Al_{94.5}Mo_{0.5}Co₅ | 380 | 100 | Duc | Comparative Example |
| 134 | Al₈₃Mo₁₅Co₂ | 510 | 410 | Bri | Comparative Example |
| 135 | Al₉₀Mo₂Co₈ | 490 | 420 | Bri | Comparative Example |
| 136 | Al_{98.5}Mo_{0.5}Co₁ | 360 | 105 | Duc | Comparative Example |
| 137 | Al₈₅Mo₁₁Co₄ | 460 | 430 | Bri | Comparative Example |
| 138 | Al_{94.5}Mo_{0.5}Cu₅ | 340 | 105 | Duc | Comparative Example |
| 139 | Al₈₈Mo₁₁Cu₁ | 490 | 430 | Bri | Comparative Example |
| 140 | Al₈₉Mo₃Cu₈ | 510 | 410 | Bri | Comparative Example |
| 141 | Al₉₈Mo₁Cu₁ | 410 | 95 | Duc | Comparative Example |
| 142 | Al₈₅Mo₁₂Cu₃ | 550 | 420 | Bri | Comparative Example |
| 143 | Al_{96.5}Fe_{0.5}Mn₃ | 420 | 130 | Duc | Comparative Example |
| 144 | Al₈₆Fe₁₂Mn₂ | 510 | 430 | Bri | Comparative Example |
| 145 | Al₉₇Fe₃ | 480 | 160 | Duc | Comparative Example |
| 146 | Al₉₀Fe₄Mn₆ | 530 | 425 | Bri | Comparative Example |
| 147 | Al₉₈Fe₁Mn₁ | 480 | 95 | Duc | Comparative Example |
| 148 | Al₈₇Fe₁₀Mn₃ | 510 | 420 | Bri | Comparative Example |
| 149 | Al_{95.5}Fe_{0.5}Ni₄ | 470 | 105 | Duc | Comparative Example |
| 150 | Al₈₆Fe₁₁Ni₃ | 510 | 420 | Bri | Comparative Example |
| 151 | Al₈₉Fe₄Ni₇ | 505 | 425 | Bri | Comparative Example |
| 152 | Al₉₈Fe₁Ni₁ | 380 | 95 | Duc | Comparative Example |
| 153 | Al₈₅Fe₁₁Ni₄ | 500 | 410 | Bri | Comparative Example |
| 154 | Al_{94.5}Fe_{0.5}Co₅ | 380 | 125 | Duc | Comparative Example |
| 155 | Al₈₃Fe₁₅Co₂ | 200 | 480 | Bri | Comparative Example |
| 156 | Al₉₀Fe₂Co₈ | 490 | 425 | Bri | Comparative Example |
| 157 | Al_{98.5}Fe_{0.5}Co₁ | 380 | 95 | Duc | Comparative Example |
| 158 | Al₈₅Fe₁₁Co₄ | 350 | 435 | Bri | Comparative Example |
| 159 | Al_{94.5}Fe_{0.5}Cu₅ | 340 | 105 | Duc | Comparative Example |
| 160 | Al₈₈Fe₁₁Cu₁ | 410 | 435 | Bri | Comparative Example |
| 161 | Al₈₉Fe₃Cu₈ | 480 | 410 | Bri | Comparative Example |
| 162 | Al₉₈Fe₁Cu₁ | 410 | 95 | Duc | Comparative Example |
| 163 | Al₈₅Fe₁₂Cu₃ | 550 | 420 | Bri | Comparative Example |
| 164 | Al_{96.5}W_{0.5}Mn₃ | 380 | 120 | Duc | Comparative Example |
| 165 | Al₈₆W₁₂Mn₂ | 420 | 435 | Bri | Comparative Example |
| 166 | Al₉₇W₃ | 280 | 95 | Duc | Comparative Example |
| 167 | Al₉₀W₄Mn₆ | 490 | 440 | Bri | Comparative Example |
| 168 | Al₉₈W₁Mn₁ | 280 | 95 | Duc | Comparative Example |
| 169 | Al₈₇W₁₀Mn₃ | 290 | 475 | Bri | Comparative Example |
| 170 | Al_{96.5}W_{0.5}Fe₃ | 385 | 105 | Duc | Comparative Example |
| 171 | Al₈₅W₁₃Fe₂ | 310 | 480 | Bri | Comparative Example |
| 172 | Al₉₈W₁Fe₁ | 320 | 105 | Duc | Comparative Example |
| 173 | Al₈₇W₁₀Fe₃ | 500 | 475 | Bri | Comparative Example |
| 174 | Al₉₀W₄Fe₆ | 510 | 460 | Bri | Comparative Example |
| 175 | Al_{95.5}W_{0.5}Ni₄ | 380 | 95 | Duc | Comparative Example |
| 176 | Al₈₆W₁₁Ni₁₃ | 520 | 470 | Bri | Comparative Example |
| 177 | Al₈₉W₄Ni₇ | 500 | 435 | Bri | Comparative Example |
| 178 | Al₉₈W₁Ni₁ | 280 | 80 | Duc | Comparative Example |
| 179 | Al₈₅W₁₁Ni₄ | 460 | 435 | Bri | Comparative Example |
| 180 | Al_{94.5}W_{0.5}Co₅ | 275 | 105 | Duc | Comparative Example |
| 181 | Al₈₃W₁₅Co₂ | 500 | 460 | Bri | Comparative Example |
| 182 | Al₉₀W₂Co₈ | 410 | 445 | Bri | Comparative Example |
| 183 | Al_{98.5}W_{0.5}Co₁ | 270 | 85 | Duc | Comparative Example |
| 184 | Al₈₅W₁₁Co₄ | 290 | 470 | Bri | Comparative Example |
| 185 | Al_{94.5}W_{0.5}Cu₅ | 340 | 105 | Duc | Comparative Example |
| 186 | Al₈₈W₁₁Cu₁ | 310 | 435 | Bri | Comparative Example |
| 187 | Al₈₉W₃Cu₈ | 380 | 410 | Bri | Comparative Example |
| 188 | Al₉₈W₁Cu₁ | 410 | 95 | Duc | Comparative Example |
| 189 | Al₈₅W₁₂Cu₃ | 550 | 420 | Bri | Comparative Example |
| 190 | Al_{96.5}Nb_{0.5}Mn₃ | 430 | 120 | Duc | Comparative Example |
| 191 | Al₈₆Nb₁₂Mn₂ | 510 | 475 | Bri | Comparative Example |
| 192 | Al₉₇Nb₃ | 430 | 105 | Duc | Comparative Example |
| 193 | Al₉₀Nb₄Mn₆ | 490 | 430 | Bri | Comparative Example |
| 194 | Al₉₈Nb₁Mn₁ | 380 | 95 | Duc | Comparative Example |
| 195 | Al₈₇Nb₁₀Mn₃ | 390 | 465 | Bri | Comparative Example |
| 196 | Al_{96.5}Nb_{0.5}Fe₃ | 400 | 95 | Duc | Comparative Example |
| 197 | Al₈₅Nb₁₃Fe₂ | 390 | 480 | Bri | Comparative Example |
| 198 | Al₉₈Nb₁Fe₁ | 430 | 100 | Duc | Comparative Example |
| 199 | Al₈₇Nb₁₀Fe₃ | 510 | 435 | Bri | Comparative Example |
| 200 | Al₉₀Nb₄Fe₆ | 420 | 80 | Bri | Comparative Example |
| 201 | Al_{95.5}Nb_{0.5}Ni₄ | 380 | 110 | Duc | Comparative Example |
| 202 | Al₈₆Nb₁₁Ni₃ | 510 | 440 | Bri | Comparative Example |
| 203 | Al₈₉Nb₄Ni₇ | 490 | 435 | Bri | Comparative Example |
| 204 | Al₉₈Nb₁Ni₁ | 230 | 80 | Duc | Comparative Example |
| 205 | Al₈₅Nb₁₁Ni₄ | 430 | 475 | Bri | Comparative Example |
| 206 | Al_{94.5}Nb_{0.5}Co₅ | 280 | 95 | Duc | Comparative Example |
| 207 | Al₈₃Nb₁₅Co₂ | 410 | 470 | Bri | Comparative Example |
| 208 | Al₉₀Nb₂Co₈ | 510 | 430 | Bri | Comparative Example |
| 209 | Al_{98.5}Nb_{0.5}Co₁ | 270 | 90 | Duc | Comparative Example |
| 210 | Al₈₅Nb₁₁Co₄ | 510 | 475 | Bri | Comparative Example |
| 211 | Al_{94.5}Nb_{0.5}Cu₅ | 340 | 105 | Duc | Comparative Example |
| 212 | Al₈₈Nb₁₁Cu₁ | 490 | 445 | Bri | Comparative Example |
| 213 | Al₈₉Nb₃Cu₈ | 475 | 410 | Bri | Comparative Example |
| 214 | Al₉₈Nb₁Cu₁ | 410 | 95 | Duc | Comparative Example |
| 215 | Al₈₅Nb₁₂Cu₃ | 550 | 420 | Bri | Comparative Example |
| 216 | Al_{96.5}Pd_{0.5}Mn₃ | 380 | 105 | Duc | Comparative Example |
| 217 | Al₈₆Pd₁₂Mn₂ | 400 | 435 | Bri | Comparative Example |
| 218 | Al₉₇Pd₃ | 410 | 95 | Duc | Comparative Example |
| 219 | Al₉₀Pd₄Mn₆ | 510 | 420 | Bri | Comparative Example |
| 220 | Al₉₈Pd₁Mn₁ | 390 | 80 | Duc | Comparative Example |
| 221 | Al₈₇Pd₁₀Mn₃ | 490 | 465 | Bri | Comparative Example |
| 222 | Al_{96.5}Pd_{0.5}Fe₃ | 300 | 95 | Duc | Comparative Example |
| 223 | Al₈₃Pd₁₃Fe₂ | 210 | 480 | Bri | Comparative Example |
| 224 | Al₉₈Pd₁Fe₁ | 290 | 105 | Duc | Comparative Example |
| 225 | Al₈₇Pd₁₀Fe₃ | 460 | 435 | Bri | Comparative Example |
| 226 | Al₉₀Pd₄Fe₆ | 475 | 430 | Bri | Comparative Example |
| 227 | Al_{95.5}Pd_{0.5}Ni₄ | 310 | 90 | Duc | Comparative Example |
| 228 | Al₈₆Pd₁₁Ni₃ | 410 | 465 | Bri | Comparative Example |
| 229 | Al₈₉Pd₄Ni₇ | 460 | 450 | Bri | Comparative Example |
| 230 | Al₉₈Pd₁Ni₁ | 280 | 85 | Duc | Comparative Example |
| 231 | Al₈₅Pd₁₁Ni₄ | 410 | 460 | Bri | Comparative Example |
| 232 | Al_{94.5}Pd_{0.5}Co₅ | 430 | 120 | Duc | Comparative Example |
| 233 | Al₈₃Pd₁₅Co₂ | 290 | 485 | Bri | Comparative Example |
| 234 | Al₉₀Pd₂Co₈ | 425 | 430 | Bri | Comparative Example |
| 235 | Al_{98.5}Pd_{0.5}Co₁ | 290 | 95 | DuC | Comparative Example |
| 236 | Al₈₅Pd₁₁Co₄ | 460 | 465 | Bri | Comparative Example |
| 237 | Al_{94.5}Pd_{0.5}Cu₅ | 340 | 105 | Duc | Comparative Example |
| 238 | Al₈₈Pd₁₁Cu₁ | 475 | 435 | Bri | Comparative Example |
| 239 | Al₈₉Pd₃Cu₈ | 490 | 410 | Bri | Comparative Example |
| 240 | Al₉₈Pd₁Cu₁ | 410 | 95 | Duc | Comparative Example |
| 241 | Al₈₅Pd₁₂Cu₃ | 550 | 420 | Bri | Comparative Example |

Samples No. 4, 5, 6, 18 and 19 of Table 1 do not form part of the invention.

It is clear from the results shown in Tables 1 and 2 that an aluminum-based alloy possessing a high bearing force and hardness, which endured bending and could undergo processing, was obtainable when the alloy comprising at least one of Mn, Fe, Co, Ni, and Cu, as element M, in addition to an Al-V, Al-Mo, Al-W, Al-Fe, Al-Nb, or Al-Pd two-component alloy has the atomic percentages satisfied the relationships Al_{balance}QₐM_{b}, 1 ≤ a ≤ 10, 0 < b < 5, 3 ≤ a+b ≤ 12, Q = V, Mo, Fe, W, Nb, and/or Pd, and M = Mn, Fe, Co, Ni, and/or Cu.

In contrast to normal aluminum-based alloys which possess an Hv of approximately 50 to 100 DPN, the samples according to the present invention, shown in Table 1, with exception of alloys wherein M is Fe when Q is V or Fe, display an extremely high hardness from 295 to 375 DPN.

In addition, in regards to the tensile rupture strength (σ_{f}), normal age hardened type aluminum-based alloys (Al-Si-Fe type) possess values from 200 to 600 MPa; however, the samples according to the present invention have clearly superior values in the range from 630 to 1350 MPa.

Furthermore, when considering that the tensile strengths of aluminum-based alloys of the AA6000 series (alloy name according to the Aluminum Association (U.S.A.)) and AA7000 series which lie in the range from 250 to 300 MPa, Fe-type structural steel sheets which possess a value of approximately 400 MPa, and high tensile strength steel sheets of Fe-type which range from 800 to 980 MPa, it is clear that the aluminum-based alloys according to the present invention display superior values.

Fig. 2 shows an X-ray diffraction pattern possessed by an alloy sample having the composition of Al₉₄V₄Fe₂. Fig. 3 shows an X-ray diffraction pattern possessed by an alloy sample having the composition of Al₉₅Mo₃Ni₂. Fig. 4 shows an X-ray diffraction pattern possessed by an alloy sample having the composition of Al₉₁Nb₆Co₃. According to these patterns, each of these three alloy samples has a multiphase structure comprising a fine Al-crystalline phase having an fcc structure and a fine regular-icosahedral quasi-crystalline phase. In these patterns, peaks expressed as (111), (200), (220), and (311) are crystalline peaks of Al having an fcc structure, while peaks expressed as (211111) and (221001) are dull peaks of regular-icosahedral quasi crystals.

Fig. 5 shows the DSC (Differential Scanning Calorimetry) curve in the case when an alloy having the composition of Al₉₄V₄Ni₂ is heated at rate of 0.67 K/s. In this figure, a dull exothermal peak, which is obtained when a quasi-crystalline phase is changed to a stable crystalline phase, is seen in the high temperature region.

## Claims

1. An aluminum-based alloy of high strength and high rigidity **characterized by** consisting of a composition represented by the general formula Al_{100-(a+b)}QₐM_{b};
wherein Q is at least one metal element selected from the group consisting of V, Mo, Fe, W, Nb, and Pd; M is at least one metal element selected from the group consisting of Mn, Fe, Co, Ni, and Cu; wherein M is not Fe when Q is V or Fe; and a and b, which represent a composition ratio in atomic percentages, satisfy the relationships 1 ≤ a ≤ 10, 1 ≤ b < 5, and 3 ≤ a+b ≤ 12;
said aluminum-based alloy having a metallographic structure comprising a quasi-crystalline phase.

2. An aluminum-based alloy of high strength and high rigidity according to Claim 1, **characterized in that** said metallographic structure is a multiphase structure comprising a quasi-crystalline phase and an aluminum phase.

3. An aluminum-based alloy of high strength and high rigidity according to Claim 1, **characterized in that** said metallographic structure is a multiphase structure comprising a quasi-crystalline phase and a metal solid solution having an aluminum matrix.

4. An aluminum-based alloy of high strength and high rigidity according to Claim 1, **characterized in that** said metallographic structure is a multiphase structure comprising a quasi-crystalline phase and a stable or metastable intermetallic compound phase.

5. An aluminum-based alloy of high strength and high rigidity according to Claim 1, **characterized in that** said metallographic structure is a multiphase structure comprising a quasi-crystalline phase, an amorphous phase, and a metal solid solution having an aluminum matrix.

6. An aluminum-based alloy of high strength and high rigidity according to one of Claims 1 to 5, **characterized in that** a+b is not more than 8.

7. An aluminum-based alloy of high strength and high rigidity according to one of Claims 1 to 5, **characterized in that** a+b is not more than 6.

8. An aluminum-based alloy of high strength and high rigidity according to one of Claims 1 to 7, **characterized in that** a is not less than 2.

9. An aluminum-based alloy of high strength and high rigidity according to one of Claims 1 to 8, **characterized in that** a is not more than 8.

10. An aluminum-based alloy of high strength and high rigidity according to one of Claims 1 to 8, **characterized in that** a is not more than 6.

11. An aluminum-based alloy of high strength and high rigidity according to one of Claims 1 to 11, **characterized in that** b is not more than 3.

12. An aluminum-based alloy of high strength and high rigidity according to one of Claims 1 to 11, **characterized in that** b is not more than 2.

13. A production method for an aluminium-based alloy of high strength and high rigidity having a metallographic structure incorporating a quasi-crystalline phase, said production method **characterized by** comprising a step selected from the group of:
the step of performing quick-quench solidification of an alloy liquid-melt, by means of a liquid quick-quenching method;
the step of forming a thin layer by using an alloy liquid-melt;
the step of quick-quenching an alloy liquid-melt by means of an atomizer method; and
the step of quick-quenching an alloy liquid-melt by means of a spray method;
said alloy liquid-melt consisting of Al having an amount in atomic percentage of 100-(a+b), element Q having an amount in atomic percentage of a, and element M having an amount in atomic percentage of b;
wherein said element Q is at least one metal element selected from the group consisting of V, Mo, Fe, W, Nb, and Pd; element M is at least one metal element selected from the group consisting of Mn, Fe, Co, Ni, and Cu;
wherein M is not Fe when Q is V or Fe; and a and b satisfy the relationships 1 ≤ a ≤ 10, 1 ≤ b < 5, and 3 ≤ a+b ≤ 12.

## Patentansprüche

1. Eine hochfeste und hochsteife Aluminium-Basislegierung, **gekennzeichnet dadurch, dass** sie aus einer Zusammensetzung besteht, die repräsentiert wird durch die allgemeine Formel Al_{100(a+b)} QₐM_{b}; wobei Q mindestens ein Metallelement ist, ausgewählt aus der Gruppe bestehend aus: V, Mo, Fe, W, Nb und Pd;
M mindestens ein Metallelement ist, ausgewählt aus der Gruppe, die aus folgendem besteht: Mn, Fe, Co, Ni und Cu;
wobei M nicht Fe ist, wenn Q V oder Fe ist; und, wobei a und b, welche ein Zusammensetzungsverhältnis in Atomprozent repräsentieren, denen Beziehungen 1 ≤ a ≤ 10, 1 ≤ b ≤ 5 und 3 ≤ a + b ≤ 12 genügen;
wobei die Aluminium-Basislegierung eine metallographische Struktur besitzt, welche eine quasi-kristalline Phase aufweist.

2. Eine hochfeste und hochsteife Aluminium-Basislegierung nach Anspruch 1, **dadurch gekennzeichnet, dass** die metallographische Struktur eine Mehr- oder Multifaserstruktur ist, und eine quasi-kristalline Phasen und eine Aluminiumphase aufweist.

3. Eine hochfeste und hochsteife Aluminlum-Basislegierung nach Anspruch 1, **dadurch gekennzeichnet, dass** die metallographische Struktur eine Muliphasenstruktur ist, die eine quasi-kristalline Phase und eine Metallfestlösung mit einer Aluminiummatrix aufweist.

4. Eine hochfeste und hochsteife Aluminium-Basislegierung nach Anspruch 1, **dadurch gekennzeichnet, dass** die metallographische Struktur eine Multiphasenstruktur ist, die eine quasi-kristalline Phase und eine stabile oder metastabile intermetallische Verbindungsphase aufweist.

5. Eine hochfeste und hochsteife Aluminium-Basislegierung nach Anspruch 1, **dadurch gekennzeichnet, dass** die metallographische Struktur eine Multiphasenstruktur ist, die eine quasi-kristalline Phase, eine amorphe Phase und eine Metallfestlösung mit einer Aluminiummatrix aufweist.

6. Eine hochfeste und hochsteife Alumlnium-Basislegierung nach einem der Ansprüche 1-5, **dadurch gekennzeichnet, dass** a + b nicht größer als 8 ist.

7. Eine hochfeste und hochsteife Aluminium-Basislegierung nach einem der Ansprüche 1-5, **dadurch gekennzeichnet, dass** a + b nicht größer als 6 ist.

8. Eine hochfeste und hochsteife Aluminium-Basislegierung nach einem Ansprüche 1-7, **dadurch gekennzeichnet, dass** a nicht kleiner als 2 ist.

9. Eine hochfeste und hochsteife Aluminium-Basislegierung nach einem der Ansprüche 1-8, **dadurch gekennzeichnet, dass** a nicht größer als 8 ist.

10. Eine hochfeste und hochsteife Aluminium-Basislegierung nach einem der Ansprüche 1-8, **dadurch gekennzeichnet, dass** a nicht größer als 6 ist.

11. Eine hochfeste und hochsteife Aluminium-Basislegierung nach einem der Ansprüche 1 - 10, **dadurch gekennzeichnet, dass** b nicht größer als 3 ist.

12. Eine hochfeste und hochsteife Aluminium-Basislegierung nach einem der Ansprüche 1-11, **dadurch gekennzeichnet, dass** b nicht größer als 2 ist.

13. Ein Herstellungsverfahren für eine eine hohe Festigkeit und hohe Starrheit besitzende, auf Aluminium basierende Legierung mit einer metallographischen Struktur, die eine quasi-kristalline Struktur besitzt, wobei das Herstellungsverfahren **gekennzeichnet ist durch** einen Schritt, ausgewählt aus der Gruppe von:
Den Schritt des Ausführens einer Schnellabkühlungsverfestigung einer Legierungsflüssigkeitsschmelze mittels eines Flüssigkeltsschnell-Abkühl- oder Abschreckverfahrens;
den Schritt des Ausbildens einer neuen Schicht unter Verwendung einer Legierungsflüssigkeitsschmelze;
den Schritt des Schnellabkühlens einer Legierungsflüssigkeitsschmelze mittels eines Atomisierungsverfahrens; und
den Schritt des Schnellabkühlens einer Legierungsflüssigkeitsschmelze mittels eines Sprühverfahrens;
wobei die Legierungsflüssigkeitsschmelze besteht aus Aluminium mit einer Menge in Atomprozent von 100 - (a + b), Element Q mit einer Menge in Atomprozent von a und Element M in Atomprozent von b;
wobei das erwähnte Element Q mindestens ein Metallelement ist, und zwar ausgewählt aus der Gruppe, die aus folgendem besteht:
V, Mo, Fe, W und Pd;
wobei das Element M wenigstens ein Metallelement ist, und zwar ausgewählt aus der Gruppe bestehend aus Mn, Fe, Co, Ni und Cu;
wobei M nicht Fe ist, wenn Q V oder Fe ist; und
wobei a und b den folgenden Beziehungen genügen: 1 ≤ a ≤ 10, 1 ≤ b < 5 und 3 ≤ a+b ≤ 12.

## Revendications

1. Alliage à base d'aluminium de grande solidité et de grande rigidité, **caractérisé en ce qu'**il a une composition représentée par la formule générale (Al_{100-(a+b)}QₐM_{b}) ;
où Q est au moins un élément métallique choisi dans le groupe comprenant V, Mo, Fe, W, Nb et Pd ; M est au moins un élément métallique choisi dans le groupe comprenant Mn, Fe, Co, Ni et Cu ; M n'étant pas Fe quand Q est V ou Fe ; et a et b, qui représentent un pourcentage atomique, satisfont aux relations 1≤a≤10, 1≤b≤5, et 3≤a+b≤12 ;
l'alliage à base d'aluminium ayant une structure métallographique comprenant une phase quasi-cristalline.

2. Alliage à base d'aluminium de grande solidité et de grande rigidité selon la revendication 1, **caractérisé en ce que** la structure métallographique est une structure multiphase comprenant une phase quasi-cristalline et une phase d'aluminium.

3. Alliage à base d'aluminium de grande solidité et de grande rigidité selon la revendication 1, **caractérisé en ce que** la structure métallographique est une structure multiphase comprenant une phase quasi-cristalline et une solution solide métallique comportant une matrice d'aluminium.

4. Alliage à base d'aluminium de grande solidité et de grande rigidité selon la revendication 1, **caractérisé en ce que** la structure métallographique est une structure multiphase comprenant une phase quasi-cristalline et une phase de composés métalliques stables ou métastables.

5. Alliage à base d'aluminium de grande solidité et de grande rigidité selon la revendication 1, **caractérisé en ce que** la structure métallographique est une structure multiphase comprenant une phase quasi cristalline, une phase amorphe et une solution solide métallique comportant une matrice d'aluminium.

6. Alliage à base d'aluminium de grande solidité et de grande rigidité selon l'une quelconque des revendications 1 à 5, **caractérisé en ce que** a+b n'est pas supérieur à 8.

7. Alliage à base d'aluminium de grande solidité et de grande rigidité selon l'une quelconque des revendications 1 à 5, **caractérisé en ce que** a+b n'est pas supérieur à 6.

8. Alliage à base d'aluminium de grande solidité et de grande rigidité selon l'une quelconque des revendications 1 à 7, **caractérisé en ce que** a n'est pas inférieur à 2.

9. Alliage à base d'aluminium de grande solidité et de grande rigidité selon l'une quelconque des revendications 1 à 8, **caractérisé en ce que** a n'est pas supérieur à 8.

10. Alliage à base d'aluminium de grande solidité et de grande rigidité selon l'une quelconque des revendications 1 à 8, **caractérisé en ce que** a n'est pas supérieur à 6.

11. Alliage à base d'aluminium de grande solidité et de grande rigidité selon l'une quelconque des revendications 1 à 11, **caractérisé en ce que** b n'est pas supérieur à 3.

12. Alliage à base d'aluminium de grande solidité et de grande rigidité selon l'une quelconque des revendications 1 à 11, **caractérisé en ce que** b n'est pas supérieur à 2.

13. Procédé de fabrication d'un alliage à base d'aluminium de grande solidité et de grande rigidité ayant une structure métallographique incorporant une phase quasi-cristalline, **caractérisé en ce qu'**il comprend une étape choisie parmi le groupe suivant :
l'étape consistant à réaliser une solidification par trempe rapide d'un alliage liquide fondu par un procédé de trempe rapide liquide ;
l'étape de formation d'une couche mince en utilisant un alliage liquide fondu ;
l'étape de trempe rapide d'un alliage liquide fondu par un procédé d'atomisation ;
l'étape de trempe rapide d'un alliage liquide fondu par un procédé de pulvérisation ;
l'alliage liquide fondu comprenant de l'aluminium en un pourcentage atomique de 100-(a+b), un élément Q dans une quantité en pourcentage atomique de a, et un élément M dans une quantité en pourcentage atomique de b ;
dans lequel l'élément Q est au moins un élément métallique choisi dans le groupe comprenant V, Mo, Fe, W, Nb et Pd ; M est au moins un élément métallique choisi dans le groupe comprenant Mn, Fe, Co, Ni et Cu ;
dans lequel M n'est pas Fe quand Q est V ou Fe ; et
a et b satisfont aux relations 1≤a≤10, 1≤b<5, et 3≤a+b≤12.
